

Aug. 10, 1937.

E. S. CORNELL, JR.

2,089,784

METHOD OF PRODUCING INTEGRAL SWEAT JOINTED ADAPTERS  
AND THE ARTICLE RESULTING THEREFROM

Filed Dec. 24, 1935

2 Sheets-Sheet 1



INVENTOR  
Edward S. Cornell, Jr.

BY  
Henry J. Hale  
HIS ATTORNEY

Aug. 10, 1937.

E. S. CORNELL, JR.  
METHOD OF PRODUCING INTEGRAL SWEAT JOINTED ADAPTERS  
AND THE ARTICLE RESULTING THEREFROM

2,089,784

Filed Dec. 24, 1935

2 Sheets-Sheet 2



INVENTOR  
Edward S. Cornell Jr.  
BY  
Henry J. Luecke  
HIS ATTORNEY

## UNITED STATES PATENT OFFICE

2,089,784

METHOD OF PRODUCING INTEGRAL  
SWEAT-JOINTED ADAPTERS AND  
THE ARTICLE RESULTING THERE-  
FROMEdward S. Cornell, Jr., Larchmont, N. Y., assignor  
to American Radiator Company, New York,  
N. Y., a corporation of New Jersey

Application December 24, 1935, Serial No. 56,031

13 Claims. (Cl. 29—157)

My present invention relates to a method of producing integral sweat-jointed adapters and the therefrom resulting adapters.

The present invention is particularly directed 5 to the production of integral adapters of copper, or of an alloy or other metallic composition predominantly of copper content, by cold working operations, that is to say, without supplied heat.

10 More particularly, as to the production of adapters of general cylindrical contour, provided with an intermediately disposed relatively thickened wall portion, bearing a hexagonal or other polygonal configuration, for application of a suitable tool, a blank conveniently a length of pipe or tube is selected of predetermined cubical content and subjected to die and punch operation, the effective recess of the die being configurated in correspondence to the final outer configuration 15 of the desired adapter, the configuration of such recess of the die in particular providing for the stated relatively thickened portion and for one end portion of sufficiently thickened wall, preferably tapered, for bearing threading, the 20 punch being subjected to forcible movement relative to the die to effect integral cold flow of the metal to final status, the derived adapter being integral and of solid wall formation throughout.

Adapters produced pursuant to my invention, 25 arranged for sweat-jointed connection, are formed at the to-be-sweated end of relatively reduced wall thickness, one face of which is substantially smooth and of uniform diameter throughout, such diameter being of a magnitude 30 relative to the diameter of the end of a pipe or of another fitting to effect a clearance affording capillary and/or surface flow of the bonding medium in fluid status under heat for effecting such sweated joint. For a female joint such 35 smooth uniform diameter face is preferably provided with a shoulder, defining such smooth face and predetermining the area of the resulting joint capable upon congealing of the bonding medium to withstand internal pressure of the 40 fluid conveyed in use, also load and other stresses incident in use, stresses arising from expansion and contraction, etc. Such reduced wall thickness advantageously corresponds to the wall 45 thickness of the end of the pipe or of another fitting, with which it is connected, to thereby effect like expansion and contraction, the congealed bonding medium applied over the predeter- 50 mined area, coating with such reduced wall

thickness to constitute a commercially rigid joint.

In commercial practice, the blank is advantageously a cylindrical annulus, which may be of uniform inner diameter and uniform outer diameter and accordingly of uniform thickness throughout, whereby in carrying out of my invention the to-be-sweated end of the blank is reduced in wall thickness by the integral cold flow of the metal from such to-be-reduced wall end 10 portion toward and eventually solidly toward and eventually as a portion of the to-be-enlarged intermediate portion to form the desired outwardly polygonal configurated portion of the adapter, and also toward and eventually as a portion of 15 the to-be-enlarged wall end portion, which may be and preferably is also convergently tapered and capable of bearing threading for threaded connection with a mating threaded end of a pipe or of another fitting. 20

If desired, the threading of the threaded end of the adapter may be effected by cold working, pursuant to my invention.

Further features and objects of the invention will be more fully understood from the following detail description and the accompanying drawings, in which 25

Fig. 1 is a side elevation, partly broken away in vertical section of a female type of sweat jointed and male threaded adapter embodying 30 my invention and produced pursuant to my invention.

Fig. 2 is a side elevation partly broken away in vertical section of a length of cylindrical annulus of cubical content of that of the adapter shown 35 in Fig. 1.

Fig. 3 is a vertical view taken through the plane of meeting of a two part, i. e. book die, illustrating an initial stage of my process, the punch being shown in elevation. 40

Fig. 4 is a view similar to Fig. 3 and illustrating an intermediate stage of my process.

Fig. 5 is a view similar to Figs. 3 and 4 and illustrates a final stage of my process. 45

Fig. 6 shows in elevation, partly broken away in vertical section, a range boiler adapter of the sweat-jointed type, produced by my cold working method and embodying the product characteristics of my invention.

Fig. 7 illustrates one form of blank having a cubical content substantially equal to the adapter of Fig. 6, into which the blank is cold wrought. 50

Figs. 8 and 9 illustrate in successive stages, comparable to the showings of Figs. 3 and 4, 55

steps of my method of cold working the blank of Fig. 7 into a final product from which the adapter of Fig. 6 is produced by threading operation.

5 Fig. 10 shows in vertical section, a threaded union of the sweat-jointed type, producible by my method and embodying the product characteristics of my invention.

Fig. 11 illustrates, similar to Figs. 3 and 8, a 10 stage of my method for producing the upper component element of the union shown in Fig. 10, whereas Fig. 12 illustrates a similar stage of my method for producing in final status by cold working the lower-and-threaded-component element of the union shown in Fig. 10.

Referring generally to the drawings, the steps of my method indicated in Figs. 2, 4, and 5 are specific to the formation of the illustrated type of female sweat jointed and male threaded adapter 20 of general cylindrical configuration; further, specific dimensional and outer configuration characteristics are shown. Therefore the type and specific characteristics depicted in the drawings serve as illustrative of commercial practice of my 25 invention with respect to all types of adapters.

Particular types of adapters embodying my invention and producible pursuant to my method, are illustrated in Figs. 1, 6, and 10.

Referring to the comparative figures, Figs. 1 30 and 2, the blank 10 is selected in cubical content and dimensional characteristics in correspondence to the cubical content and final dimensional characteristics of the adapter to be produced therefrom, namely, that illustrated in Fig. 1. Accordingly, its length, indicated by the double 35 arrowed dotted line 10a, corresponds to the length indicated by the double arrowed dotted line 11a, of the desired adapter 11; its inner diameter indicated by the double arrowed dotted line 40 10b, corresponds to the inner diameter indicated by the double arrowed dotted line 11b, of the threaded end 11c of the adapter 11, and its cubical content, i. e., its outer diameter and its 45 wall thickness, corresponds to the cubical content of the desired adapter 11.

Such length of blank, i. e., cylindrical annulus 10 is placed in a suitable die, conveniently a two part die 12, usually of the book type, the effective cavity of which is configurated in correspondence 50 to the configuration of the desired adapter in final status, such cavity including the entrance bore 12a leading to the cavity portion indicated at 12b of a diameter closely approximating the outer diameter of the blank 10 and also the outer 55 diameter indicated by the double arrowed dotted line 11d, 11d, of the sweat-jointed end of the desired adapter, as shown in Fig. 1. Such die cavity further includes the intermediately disposed enlarged recess portion indicated at 12c, 60 see Fig. 3, in correspondence to the configuration of the desired hexagonal or other polygonal enlargement, see 11e, Fig. 1. Preferably, also, the effective cavity of the die includes the terminal recess portion indicated at 12d, see Fig. 3, for 65 applying a tapered terminal end as may be desired and as indicated at 11f in Fig. 1.

The die cavity preferably further comprises the recess portion indicated at 12e, corresponding to a graduate'y thickened wall portion 11h, at which 70 the threading 11c is formed, which graduate'y thickened wall portion tapers convergently toward the initial thread i. e., terminus of the threaded end portion of the adapter.

The punch 13 includes in essence a nose portion 13a, serving as a mandrel, having an outer

diameter most closely approximating the inner diameter 11b of the threaded end of the adapter, and therefore of close approximation of the inner diameter 10b of the length of the tube 10. The punch comprises further an intermediate body 5 portion 13b immediately adjacent its stated mandrel portion 13a, the outer diameter of the portion 13b corresponding to the inner diameter of the sweat jointed end, indicated by the double arrowed dotted line 11g, shown in Fig. 1. Such 10 enlargement of dimension of the punch portion 13b, relative to the punch portion 13a gives rise to the shoulder or abutment 13c. The punch comprises further the portion 13d of relatively enlarged diameter as compared with and immediately succeeding the stated punch portion 13b, thus giving rise to the shoulder or abutment 13e. The diameter of the punch portion 13d most closely approximates the diameter of the entrance bore 12a of the die. The diameter of the 20 free end portion 13a of the punch most closely approximates the diameter of the lower bore 12f of the die.

Upon application of suitable force upon the head 13f of the punch, forcibly causing the punch 25 to be displaced relative to the die 12, as is indicated in Fig. 4, the stated shoulder 13c effects a flow of metal at the to-be-sweat-jointed end 11j of the blank 10, the shoulder 13c in co-operation with the mandrel portion 13a effecting a solid 30 flow of the metal and gradually and integrally flowing into the enlarged recess portion 12c, tending toward the formation as a solid wall the relatively thickened portion bearing the hexagonal or other polygonal configuration 11e. 35

Fig. 4 also illustrates the similar cold flow as an ever integral and ever solid mass of the metal into the lowerly tapered cavity recess 12d, toward or fully effecting the tapered end periphery 11f of the adapter 11, usually and preferably 40 desired.

Upon continuation of the stated force upon the punch to final position, indicated in Fig. 5, the stated cold wrought flow of the metal consummates the desired internal and external configurations and desired differential wall thicknesses of the ultimate adapter. It is observed that additive to the stated functions the shoulder 13c of the punch effects the formation of a correspondingly contoured shoulder 11k of the adapter, 50 desirable in a type of female sweat-jointed adapter, such as is shown in Fig. 1. Further, it is observed that the shoulder 13e of the punch serves the dual functions of guiding, and limiting the upward extent of, the flow of metal in the 55 clearance between the punch portion 13b and the entrance bore 12a of the die and eventually to determine and finish the terminal portion of the sweat-jointed end 11j of the adapter.

Preferably, as is shown in Fig. 3, the extent of 60 movement of the punch 13 into the bore of the die is positively safeguarded by the provision of the shoulder 13g, had by suitable enlargement of the body of the head 13f of the punch, which shoulder 13g may be arcuate in correspondence 65 to the arcuate terminus 12g of the entrance bore of the die.

Upon completion of the stated or equivalent operations, the produced product i. e. adapter, minus threads in this instance, is removed from 70 the die, the punch being withdrawn, and the threading then produced by suitable tapping, as will be understood.

In the stated procedure, the whole of the cubical content of the cylindrical annulus 10 has been 75

preserved in the formation of the adapter 11, compare Fig. 1 with Fig. 2, excepting for the removal of metal ensuing in the threading operation.

- 5 As appears, the desired threading may be had by intaglio thread contouring the recess portion 12e of the die cavity to cause cold integral flow of the metal similarly as above described, into such intaglio thread formations.
- 10 Fig. 6 illustrates another type of adapter, and Figs. 7, 8, and 9 illustrate my method, pursuant to the aforesaid essential steps, for producing the adapter shown in Fig. 6. The adapter 15 shown in Fig. 6 is a component of a type of range boiler fitting and comprises at one end 15j having an inner face of uniform diameter 15g, and smooth throughout, and of a predetermined area and arranged for sweat-connected connection for an end of a pipe or the like. The opposite end 15c of the 20 fitting at both its inner and outer faces is provided with threading, the threading at its outer face being designated 15c' and at its inner face 15c''. The wall 15h of such threaded end 15c is suitably thickened to receive and bear such 25 double threading. Intermediate the ends of the adapter 15 its solid wall 15h is further thickened, see 15h', to extend laterally of the mean width of the adapter, to bear a polygonal configuration 15e. Advantageously, as shown in Fig. 6, 30 the thickened wall portion 15h' of the polygonal configuration 15e, merges with the thick wall portion 15h, bearing the threading 15c', 15c''.

The outer threading 15c' may mesh with a threaded opening in a range boiler and the inner 35 threading 15c'' may mesh with a threaded end of a pipe or the like.

Such adapter 15, pursuant to my invention, may be formed from a blank 16, see Figs. 7 and 8, having a predetermined cubical content corresponding to that of the resulting adapter 15, and of predetermined inner and outer diameter, and resulting wall thickness corresponding to a mean wall thickness of, say, the doubly threaded end 15c of the eventual adapter. As one economical 45 manner of carrying out such form of my method, see Figs. 8 and 9, such blank 16 is cold worked and subjected to integral cold flow in a book die 11, provided with an entrance bore 17a, a recess 17b corresponding to the desired enlargement of the wall formation of the polygonally 50 configured portion 15e; further, with a recess 17c corresponding to the wall formation of the to-be-sweat-connected end 15j, and further with a lower bore 17b. The punch 13 corresponds 55 generally (but of lesser number of step formations) to the aforesaid punch indicated in Figs. 3, 4, and 5; like parts are designated by like reference characters. Fig. 8 shows the preliminary stage of placement of the blank 16 with the recess 60 portion of the die and the punch 13 placed in the entrance bore 17a. Fig. 9 shows the concluding stage of the displacement of the punch 13 and consequent cold working and integral cold flow of the metal into the desired final formation of the adapter 15, preparatory for threading interiorly and exteriorly corresponding to the threading 15c'', 15c'.

In Fig. 10 is illustrated other embodiments 70 pursuant to my invention. The particular structure illustrated in Fig. 10 is of the threaded union type, the upper component 18 having its upper end 18j adapted, viz. on its inner face, to be sweat-jointed at its inner face to an end of a 75 pipe or the like, and of uniform diameter, smooth

faced and of predetermined area, similarly as above, its lower end being thickened in wall, see 18h. For particular assembly and utility as a component of a union, the lower face 18k is convergently tapered in the downward direction, to 5 serve as a compression face, as will appear.

Cooperating with such upper component 18, of such threaded union assembly, is shown in Fig. 10, the lower component 19 having at its upper end an enlarged wall formation 19h, provided at its upper terminus with a face formation 19k divergently tapered in upward direction, corresponding to the stated convergently tapered face formation 18k, to form a compression joint thereat. The upper enlarged wall formation 19h is also provided with threading 19c, mating with the threading on the inner face of the nut 20, completing the threaded union assembly, the diameter of the wall 20a of the upper opening of the nut 20 being less than the outer diameter 20 of the enlarged lower wall formation 18h of the upper component 18.

The lower component 19 further comprises at its end 19j a face, i. e., its inner face in this instance, which is smooth, of uniform diameter, 25 and predetermined in area by the shoulder 19k, arranged for sweat-connection with an end of a pipe or the like.

The upper component 18, pursuant to my method, may be formed from an annular blank 21, 30 shown positioned in the cavity of the die 22, such cavity including a recess enlargement 22a and a lowerly recess formation 22b corresponding to the final formation of the lower end of the upper component 18, the metal of the blank 21 being 35 subjected to integral cold flow by the operation of the punch 13, which may correspond to the aforesaid punch shown in Figs. 3, 4, and 5. Like parts are designated by like reference characters. Upon forced movement of such punch 13, 40 to its lower position indicated by the dot-and-dash line 22c, integral cold flow of the metal ensues, similarly as above.

The lower component 19, of the threaded union shown in Fig. 10, pursuant to my invention may 45 be similarly formed of a blank 23 shown in position in the die 24, see Fig. 12, the punch 13 corresponding to the punch 13 shown in Figs. 3, 4, and 5, like parts are designated by like reference characters.

In the cavity of the die 24, the recess formation 24a corresponds to the solid enlarged wall of the enlarged wall formation 19h of the component 19 shown in Fig. 10 and also embodies intaglio thread formations peripherally of the inner wall 55 thereof, whereby upon forced operation of the punch 13 downwardly within the operating bore of the die 24, namely to its position indicated by the dot-and-dash line 24b, the metal of the blank 23 is subjected to integral cold flow to effect the 60 desired final wall formation, inclusive of the threading, see 19c, by the intaglio thread formation of the die recess 24a.

By such integral cold flow of the metal, particularly of predominant copper content, the resulting metal possesses superior tensile strength, superior degree of hardness, immunity from oxidation and/or other deterioration arising from contact with water, liquids and/or gases of the nature of water within the range of atmospheric 70 temperatures, thermal heating media, domestic and industrial water supplies, refrigeration agents, etc., applicable in the major fields of the more common types of conveyed liquids.

Whereas I have described my invention by ref- 75

erence to specific forms thereof, it will be understood that many changes and modifications may be made without departing from the spirit of the invention.

5 I claim:

1. The method of producing integral adapters of wrought metal of predominant copper content, said adapter including an end portion of relatively reduced thickness having a face substantially smooth and of a substantially uniform diameter, said adapter further having an end portion of relatively large wall thickness capable of bearing a threading, said adapter further having a wall portion of relatively enlarged wall thickness bearing an outer configuration of polygonal contour, said method comprising subjecting a blank of substantially cylindrical annulus of metal of predominant copper content to punch and die operation to effect cold flow integral movement of the metal from one end portion of the annulus to reduce the wall thickness thereof and to form a face of substantially uniform diameter thereat, and guiding and limiting such cold flow integrally outwardly of the outer diametrical configuration of the original blank to produce an enlarged solid wall formation of the desired polygonal configuration, and guiding and limiting such cold flow integrally to form an enlarged solid end portion capable of bearing threading.
2. The method of producing integral adapters of wrought metal of predominant copper content, said adapter including an end portion of relatively reduced thickness having a face substantially smooth and of a substantially uniform diameter, said adapter further having an end portion of relatively large wall thickness capable of bearing a threading, said adapter further having a wall portion of relatively enlarged wall thickness bearing an outer configuration of polygonal contour, said method comprising subjecting a blank of substantially cylindrical annulus of metal of predominant copper content to punch and die operation to effect cold flow integral movement of the metal inwardly from one end portion of the annulus to reduce the wall thickness thereof and to form a face of substantially uniform diameter thereat, and guiding and limiting such cold flow integrally outwardly of the outer diametrical configuration of the original blank to produce an enlarged solid wall formation of the desired polygonal configuration, and guiding and limiting such cold flow integrally to form an enlarged solid end portion capable of bearing threading.
3. The method of producing integral adapters of wrought metal of predominant copper content, said adapter including an end portion of relatively reduced thickness having a face substantially smooth and of a substantially uniform diameter, said adapter further having an end portion of relatively large wall thickness capable of bearing a threading, said adapter further having a wall portion of relatively enlarged wall thickness bearing an outer configuration of polygonal contour, said method comprising subjecting a blank of substantially cylindrical annulus of metal of predominant copper content to punch and die operation to effect cold flow integral movement of the metal from one end portion of the annulus to reduce the wall thickness thereof and to form a face of substantially uniform diameter thereat, and guiding and limiting such cold flow integrally outwardly of the outer diametrical configuration of the original blank to produce an enlarged solid wall formation of the desired polygonal configuration, and guiding and limiting such cold flow integrally to form an enlarged solid end portion capable of bearing threading.

5 integrally to form an enlarged solid end portion capable of bearing threading, said enlarged end portion having a wall dimension less than the wall dimension of said polygonally configurated enlarged portion.

4. The method of producing integral adapters of wrought metal of predominant copper content, said adapter including an end portion of relatively reduced thickness having a face substantially smooth and of a substantially uniform 10 diameter, said adapter further having an end portion of relatively large wall thickness capable of bearing a threading, said adapter further having a wall portion of relatively enlarged wall thickness bearing an outer configuration of polygonal 15 contour, said method comprising subjecting a blank of substantially cylindrical annulus of metal of predominant copper content to punch and die operation to effect cold flow integral movement of the metal from one end portion of 20 the annulus to reduce the wall thickness thereof and to form a face of substantially uniform diameter thereat, and guiding and limiting such cold flow integrally outwardly of the outer diametrical configuration of the original blank to 25 produce an enlarged solid wall formation of the desired polygonal configuration, and guiding and limiting such cold flow integrally to form an enlarged solid end portion and having a convergingly tapered terminus capable of bearing thread- 30 ing.

5. The method of producing integral adapters of wrought metal of predominant copper content, said adapter including an end portion of relatively reduced thickness having a face substantially smooth and of a substantially uniform 35 diameter, said adapter further having an end portion of relatively large wall thickness capable of bearing a threading, said adapter further having a wall portion of relatively enlarged wall 40 thickness bearing an outer configuration of polygonal contour, said method comprising subjecting a blank of substantially cylindrical annulus of metal of predominant copper content to punch and die operation to effect cold flow integral 45 movement of the metal from one end portion of the annulus to reduce the wall thickness thereof and to form a face of substantially uniform diameter thereat, and guiding and limiting such cold flow integrally outwardly of the outer 50 diametrical configuration of the original blank to produce an enlarged tapered solid wall formation of the desired polygonal configuration, and guiding and limiting such cold flow integrally to form an enlarged solid end portion capable of 55 bearing threading.

6. The method of producing integral adapters of wrought metal of predominant copper content, said adapter including an end portion of relatively reduced thickness having a face substantially smooth and of a substantially uniform 60 diameter, said adapter further having an end portion of relatively large wall thickness capable of bearing a threading, said method comprising subjecting a blank of substantially cylindrical annulus of metal of predominant copper content to punch and die operation to effect cold flow integral 65 movement of the metal from one end portion of the annulus to reduce the wall thickness thereof and to form a face of substantially uniform diameter thereat, and guiding and limiting such cold flow integrally to form an enlarged solid end portion capable of bearing threading.

7. The method of producing integral adapters of wrought metal of predominant copper con- 75

- tent, said adapter including an end portion of relatively reduced thickness having a face substantially smooth and of a substantially uniform diameter, said adapter further having an end 5 portion of relatively large wall thickness capable of bearing a threading, said method comprising subjecting a blank of substantially cylindrical annulus of metal of predominant copper content to punch and die operation to effect cold flow 10 integral movement of the metal inwardly from one end portion of the annulus to reduce the wall thickness thereof and to form a face of substantially uniform diameter therat, and guiding and limiting such cold flow integrally to form 15 an enlarged solid end portion capable of bearing threading.
8. An adapter of cold wrought integral metal, predominately of copper content, having one of its ends provided with threading, the wall of such 20 threaded end having a thickness capable of bearing the threading when threaded to another mating threaded part, said adapter further having an end a face of which is of predetermined area and smooth and of uniform diameter throughout 25 such predetermined area, the wall of said end being solid throughout, said adapter having further a portion spaced from said smooth faced end portion having a thickened wall bearing on its outer face a polygonal configuration adapted 30 to be engaged by a suitable tool and capable of withstanding stresses incident to the use of such tool, the aforesaid adapter having superior tensile strength, superior hardness, and immunity from oxidation in use, said form and qualities 35 resulting from subjecting a substantially cylindrical blank of metal of predominant copper content to punch and die operation to effect cold flow integral movement of the metal of the blank.
9. An adapter of cold wrought integral metal, 40 predominately of copper content, having one of its ends provided with threading, the wall of such threaded end being solid throughout and having a thickness capable of bearing the threading when threaded to another mating threaded part, said adapter further having an end a face of 45 which is of predetermined area and smooth and of uniform diameter throughout such predetermined area, the wall of said smooth faced end being solid throughout, said adapter having fur- 50 ther a portion disposed intermediate its said threaded end and its said smooth faced end having a thickened wall bearing on its outer face a polygonal configuration adapted to be engaged by a suitable tool and capable of with- 55 standing stresses incident to the use of such tool, the aforesaid adapter having superior tensile strength, superior hardness, and immunity from oxidation in use, said form and qualities resulting from subjecting a substantially cylindrical 60 blank of metal of predominant copper content to punch and die operation to effect cold flow integral movement of the metal of the blank.
10. An adapter of cold wrought integral metal predominately of copper content, having one of 65 its ends provided with internally disposed threading, the wall of such threaded end having a thickness capable of bearing the threading when threaded to another mating threaded part, said adapter further having an end a face of which 70 is of predetermined area and smooth and of uniform diameter throughout such predetermined area, said adapter having further a portion the wall of said end being solid throughout bearing on its outer face a polygonal configuration adapted to be engaged by a suitable tool and 75
- capable of withstanding stresses incident to the use of such tool, the aforesaid adapter having superior tensile strength, superior hardness, and immunity from oxidation in use, said form and qualities resulting from subjecting a substantially cylindrical blank of metal of predominant copper content to punch and die operation to effect cold flow integral movement of the metal of the blank.
11. An adapter of cold wrought integral metal predominantly of copper content, having one of its ends provided with internally disposed threading, the wall of such threaded end having a thickness capable of bearing the threading when threaded to another mating threaded part, said adapter further having an end a face of which is of predetermined area and smooth and of uniform diameter throughout such predetermined area, said adapter having further a portion disposed intermediate its said threaded end and its said smooth faced end having a thickened wall bearing on its outer face a polygonal configuration adapted to be engaged by a suitable tool and capable of withstanding stresses incident to the use of such tool, the walls of said threaded end and of said smooth faced end and of said thickened wall portion being solid throughout, the aforesaid adapter having superior tensile strength, superior hardness, and immunity from oxidation in use, said form and qualities resulting from subjecting a substantially cylindrical blank of metal of predominant copper content to punch and die operation to effect cold flow integral movement of the metal of the blank.
12. An adapter of cold wrought integral metal, having one of its ends provided with internally disposed threading, the wall of such threaded end having a thickness capable of bearing the threading when threaded to another mating threaded part, said adapter further having an end an inner face of which is smooth throughout and of uniform diameter, said adapter having further a portion coincident with the wall of said internally threaded end and bearing on its outer face a polygonal configuration adapted to be engaged by a suitable tool and capable of withstanding stresses incident to the use of such tool, and a shoulder formed inwardly of and integrally with the wall of the adapter for predetermining the area of said smooth and uniform diameter face, the walls of said threaded end and of said smooth faced end and of said thickened wall portion being solid throughout, the aforesaid adapter having superior tensile strength, superior hardness, and immunity from oxidation in use, said form and qualities resulting from subjecting a substantially cylindrical blank of metal of predominant copper content to punch and die operation to effect cold flow integral movement of the metal of the blank.
13. An adapter of cold wrought integral metal predominantly of copper content, having one of its ends provided with threading, the wall of such threaded end having a thickness capable of bearing the threading when threaded to another mating threaded part, said adapter further having an end a face of which is smooth throughout and of uniform diameter, said adapter having further a portion spaced from said smooth faced end portion having a thickened wall bearing on its outer face a polygonal configuration adapted to be engaged by a suitable tool and capable of withstanding stresses incident to the use of such tool, and a shoulder formed inwardly

of and integrally with the wall of the adapter for predetermining the area of said smooth and uniform diametered face, the walls of said threaded end and of said smooth faced end and of said thickened wall portion being solid throughout, the aforesaid adapter having superior tensile strength, superior hardness, and immunity from

oxidation in use, said form and qualities resulting from subjecting a substantially cylindrical blank of metal of predominant copper content to punch and die operation to effect cold flow integral movement of the metal of the blank. 5

EDWARD S. CORNELL, JR.